

# United States Patent Office

3,167,429

Patented Jan. 26, 1965

1

3,167,429

MONOBATHS CONTAINING SODIUM POLYACRYLATE AND POLYVINYL-PYRROLIDONE  
Marilyn Levy, Red Bank, N.J., assignor to the United States of America as represented by the Secretary of the Army  
No Drawing. Filed May 26, 1961, Ser. No. 113,041  
3 Claims. (Cl. 96—61)  
(Granted under Title 35, U.S. Code (1952), sec. 266)

The invention described herein may be manufactured and used by or for the Government for governmental purposes, without the payment of any royalty thereon.

This invention relates to a one step processing formula for simultaneous development and fixing of photo-sensitive materials and particularly to such compositions for use at relatively high temperature and containing additives to increase the viscosity thereof.

In a copending patent application filed in the United States Patent Office on August 5, 1957, Serial No. 676,445, now abandoned, in which the applicant is coinventor with Willard C. Burner, a single step processing composition for photo-sensitive materials is presented. This bath produces excellent results and creates images having normal density values without excessive fog density and without decrease in film speed. In the present invention the advantages of such a bath are enlarged to apply to those special cases where the bath must have substantial viscosity to avoid spilling. For example, in airborne processing or in the operation of mobile ground processing laboratories. It has been found however when viscous monobaths are used to process photo-sensitive materials the silver that precipitates from the reaction of the monobath on exposed silver halide has a tendency to produce a cloudy veil that obscures the developed image. Such a condition is intolerable for critical applications. It so happens where processing equipment is subject to tipping and irregular displacement, as above suggested, the additional requirement for fast processing may also be present particularly in military operations wherein this additional requirement results from the urgency to view the finished picture as soon as possible. Fast processing also is urgent where the image must be immediately scanned for transmission to a remote point or to quickly supply data to data processing systems.

An effective manner for decreasing processing time is to increase the temperature of the bath. By so doing however the clouding tendency is increased. Heretofore ammonia salts have been added to the composition to correct this difficulty in which case the silver is dissolved which clears the cloudy condition. However the ammonia decreases the activity of the developer ingredients in the monobath and increases the rate of fixation to the point where both speed and maximum density in the finished image are seriously reduced. In addition the ammonia fumes released produce a toxic atmosphere.

In the practice of the invention the above difficulties are overcome. The formulation of the invention includes the developing and fixing elements of an efficient rapid acting low fogging monobath the ingredients of which are given in examples of the invention presented hereinafter. In addition to the developing and fixing ingredients a thickening agent is added such as sodium polyacrylate. More or less of this material is added depending upon the viscosity desired. To this composition is added a small quantity of polyvinylpyrrolidone. This bath is stable and can be used at temperatures up to 130° F. producing no cloudy silver precipitate.

An investigation of the mechanism producing this valuable result tends to show that the silver precipitate is kept in a transparent colloidal suspension by the polyvinyl-

2

pyrrolidone which acts as a protective colloid. The polyvinylpyrrolidone does not dissolve in the bath but remains in a suspension that is visible as microscopic droplets when viewed thru a microscope.

On the other hand, the monobath may have sufficient viscosity to be applied to the sensitive material in a thin layer by spreading it with a spatula or squeegee or by rolling it onto the emulsion. The latter technique may be carried out independently of any adverse positional environment. This high viscosity technique lends itself to a completely mechanized non-spilling processing system for rapid handling and processing of photographic materials.

The exposed sensitive material is maintained in contact with the monobath until the image is entirely cleared. At 130° F. the processing time may be 10 seconds depending on the film. The picture is then ready for immediate use. If desired subsequent washing and drying steps may be performed to prolong the initial characteristics of the image.

The following examples of solutions embodying the invention have been found to produce high quality images free of excess fog density and clouding precipitate. Also the images so processed exhibit normal density values with no indication of reduced emulsion speed.

| Example                                                 | 1   | 2   | 3   | 4   | 5   |
|---------------------------------------------------------|-----|-----|-----|-----|-----|
| Sodium polyacrylate 12.5% solution                      |     |     |     |     |     |
| 30 Sodium Sulfite cc.                                   | 550 | 650 | 550 | 700 | 500 |
| Sodium Hydroxide gm.                                    | 50  | 60  | 50  | 60  | 50  |
| Hydroquinone gm.                                        | 30  | 30  | 30  | 30  | 30  |
| 1-phenyl-3-pyrazolidone gm.                             | 25  | 25  | 25  | 25  | 25  |
| Sodium Thiosulphate gm.                                 | 3   | 3   | 3   | 3   | 3   |
| 35 Polystyrene gm.                                      | 250 | 250 | 250 | 200 | 150 |
| Polyvinylpyrrolidone gm.                                | 3   | 10  | 5   | 15  | 2   |
| Alum gm.                                                |     | 10  |     |     | 10  |
| 35 Alkyl Trimethyl ammonium chloride (50% solution) cc. |     |     | 1   |     | 1   |
| Formaldehyde 38% cc.                                    |     |     |     | 10  |     |

### Example 6

40 Water to make 1 liter.  
A quantity of chemically inactive thickening material.  
Metol gm. 10  
Sodium sulphite (anh.) gm. 50  
Hydroquinone gm. 40  
45 Potassium alum gm. 20  
Sodium hydroxide gm. 35  
Sodium thiosulphate gm. 110  
.5% solution of 6-nitrobenzimidazole nitrate cc. 20  
Polyvinylpyrrolidone gm. 10

### Example 7

Water to make 1 liter.  
A quantity of chemically inactive thickening material.  
Sodium sulphite (anh.) gm. 60  
55 1-phenyl-3-pyrazolidone gm. .8  
Hydroquinone gm. 30  
Sodium thiosulphate gm. 75 to 250  
Formaldehyde (38%) cc. 10  
Ethylene diamine 77% cc. 2 to 50  
60 Polyvinylpyrrolidone gm. 3 to 15

### Example 8

Water to make 1 liter.  
A quantity of chemically inactive thickening material.  
Sodium sulphite (anh.) gm. 50  
65 Diaminophenol hydrochloride gm. 15  
Hydroquinone gm. 5  
Glycin gm. 10  
6-nitrobenzimidazole nitrate .5% sol. cc. 80  
Sodium hydroxide gm. 20  
Ammonium thiosulphate gm. 50  
Polyvinylpyrrolidone gm. 10

The specific quantities of ingredients indicated in the above examples are not to be construed as limiting the range of quantities embraced by the invention. The useful ranges of these quantities may be expanded as set forth in the appended claims.

What is claimed is:

1. A one step processing bath for exposed silver halide photosensitive materials comprising developing elements including 1-phenyl-3-pyrazolidone and fixing agents in proportion to provide simultaneous complete development and fixing of the image and 400 to 1000 cc. of 12.5% solution sodium polyacrylate and 3 to 15 grams of polyvinylpyrrolidone per liter of solution. 10

2. A one step processing bath for exposed silver halide photosensitive material comprising:

Sodium polyacrylate 12.5% solution cc 400 to 750  
 Sodium sulphite (anhyd.) gm 40 to 70  
 Hydroquinone gm 25 to 100  
 Sodium hydroxide gm 15 to 40  
 1-phenyl-3-pyrazolidone gm .8 to 5  
 Sodium thiosulphate gm 100 to 300  
 Polyvinyl pyrrolidone gm 3 to 15  
 Formaldehyde 38% cc 0 to 20 20

3. A one step processing bath for exposed silver halide photosensitive materials containing a quantity of sodium polyacrylate as thickening material and containing the following ingredients:

Water to make 1 liter.

|                                      |    |           |
|--------------------------------------|----|-----------|
| Metol                                | gm | 5 to 15   |
| Sodium sulphite                      | gm | 40 to 70  |
| Hydroquinone                         | gm | 25 to 100 |
| 5 Potassium alum                     | gm | 10 to 30  |
| Sodium hydroxide                     | gm | 20 to 40  |
| Sodium thiosulphate                  | gm | 50 to 150 |
| Polyvinyl pyrrolidone                | cc | 3 to 15   |
| .5% solution of 6-nitrobenzimidazole | cc | 15 to 30  |

#### References Cited by the Examiner

##### UNITED STATES PATENTS

|           |       |                   |          |
|-----------|-------|-------------------|----------|
| 2,543,181 | 2/51  | Land              | 96-29    |
| 2,658,045 | 11/53 | Schildknecht      | 96-114   |
| 2,834,676 | 5/58  | Stanley et al.    |          |
| 2,875,052 | 2/59  | Weyde             | 96-114 X |
| 2,901,350 | 8/59  | Goldhammer        |          |
| 2,948,614 | 8/60  | Allen et al.      | 96-109   |
| 3,058,826 | 10/62 | Meerkamper et al. |          |

##### OTHER REFERENCES

Keelan: Photographic Engineering, vol. 4, No. 3 (1953), pages 157-161.

Keelan: Journal of Photographic Science, vol. 5 (1957), 25 pages 144-145.

NORMAN G. TORCHIN, Primary Examiner.

PHILIP E. MANGAN, Examiner.